

Patented May 17, 1927.

1,628,646

# UNITED STATES PATENT OFFICE.

ARMAN E. BECKER, OF ELIZABETH, NEW JERSEY, ASSIGNOR TO STANDARD DEVELOPMENT COMPANY, A CORPORATION OF DELAWARE.

## LUBRICANT AND PROCESS OF MAKING THE SAME.

No Drawing.

Application filed November 21, 1924. Serial No. 751,401.

This invention relates to improvements in lubricants of the type comprising an oleaginous material, especially of the petroleum type, and a soap. The invention 5 includes compositions containing in general relatively small percentages by weight of soap and relates to processes for preparing such compositions.

Various soaps may be employed in practicing my invention. In general it may be said that the saponaceous compounds of fatty acids with metals are suitable, particularly the stearates, oleates or parmitates of the alkali or alkaline earth metals 15 (referred to generically as alkali soaps).

The oil used in the present invention is preferably a good grade of lubricating oil derived from petroleum or other mineral source. However, vegetable oils or other 20 may be used for some purposes. A preferred composition consists essentially of a petroleum lubricating oil containing an alkali metal-fatty acid soap in amount less than 1/2% by weight of the oil.

25 The following is an illustration of the effect of adding small amounts of alkali metal soaps of stearic acid, oleic acid, and the like. A lubricating oil of 285 viscosity (Saybolt) at 100° F., with which was 30 incorporate 1/8% of a hard, white soap of substantial purity, tested on an Olsen friction machine at a total feed rate of 40 drops per minute, showed a friction of 5 up to 6 lbs. only, with bearing pressures from 25 up to 175 lbs. per square inch, and the revolutions per minute from 300 up to 710, and the bearing temperature from 86° F. up to 119° F. The same lubricating oil without the soap at the same total feed rate of 40 drops per minute, showed a friction of 8 up to 11.5 lbs. with bearing pressures from 25 up to 100 lbs. per square inch, and 300 revolutions per minute and bearing temperatures from 88° F. up to 108° F.

45 This improvement is believed to be due to the action of the soap in increasing the power of the oil to maintain a lubricating film. This is accomplished with minimal amounts of soap and without changing the 50 order of viscosity of the original oil. For example, in the composition referred to above, the viscosity of the oil may be increased, by the addition of the soap, from 285 to about 340 seconds Saybolt at 100° F. Such an increase does not undesirably

affect the viscosity; that is, it does not make a grease or a "bodied-up" oil too heavy for good use in the crank case of an automobile.

In preparing the improved lubricating compositions, it is generally desirable to heat the mixture of oil and soap. Solution of the soap is facilitated in this way and there is no appreciable subsequent tendency to separation, which is sometimes an objection to compositions prepared by admixture without heating. Temperatures up to the boiling point of the oil are permissible, though lower temperatures will, in general suffice. For example, in making up a composition containing lubricating oil of about 285 Saybolt viscosity at 100° F., and a sodium soap in solid condition, I prefer to heat to about 450° F. The soap may be in finely divided condition when added to the oil.

55 I have found that it is advantageous in many cases to form the soap in the body of oil by adding thereto the desired base and fatty acid in substantially combining proportions. When proceeding in this way it is possible to secure the desired result at a temperature of 350° to 375° F. This reduction of temperature, as compared with that necessary to secure the solution of a 60 preformed soap, is of large importance. Among the principal advantages of working at relatively low temperatures are the avoidance of discoloring of the oil and the reduced fire risk in making up the composition.

65 Alternatively the soap may be introduced into the oil in water solution. When working in this way temperatures in excess of 375° F. are not ordinarily required. The 70 water passes off readily during the heating and causes no difficulty. I regard the use of water-containing soaps in making up oil-soap compositions of the kind described, as an important and novel feature. Heretofore it has ordinarily been considered that the soaps used for such purpose, whether preformed or formed in situ, must be anhydrous if good results are to be obtained. My 75 experiments show that this is not the case; on the contrary there is considerable advantage in using aqueous solutions on account of the lowered temperature at which the composition may be prepared. No particular 80 strength of soap solution is necessary;

10% solutions are in general satisfactory.

When using a fatty acid, such as oleic acid, and caustic soda in forming the soap in the oil, it is generally satisfactory to use 5 these materials in chemically equivalent amounts. If a saponifiable oil, for example corn oil, is to be used instead of the fatty acid, I prefer to have the saponifiable oil present in some excess.

10 Another way in which the invention may be carried out involves the preparation of a concentrated solution or gel of soap in oil. 1% or more of the soap, which may be in solid form or in solution, may be incorporated 15 in the oil to form a stiff gelatinous mass. The proper amount of the concentrated solution may then be mixed with a suitable lubricating oil. The mixing should be thorough and should be conducted in the 20 absence of air to prevent the formation of an emulsion.

I am aware that lubricating greases, etc., have been made in which lime soaps, soda soaps and the like have been ingredients, 25 but in these the proportion of soap has been large and the consistency of the composition has been designedly increased thereby. My invention, on the other hand, is connected with a function not previously known, viz., 30 the increasing of the film-maintaining property of a lubricating oil by the addition of soaps, and this result is attained with minimal proportions and thus altogether without undesirably affecting the viscosity limits 35 and the ash content of the oil, matters which are of great importance.

The invention is not limited to the specific details given by way of illustration, and various changes may be made within the 40 scope of the appended claims.

The present application is a continuation-in-part of my copending application, Serial No. 593,906, filed October 11, 1922.

I claim:

45 1. In a process of making a lubricating oil composition, the steps of adding to a hydrocarbon oil, having lubricating properties, an effective amount of soap, less than

1/2% by weight of the oil, and heating the mixture to a temperature above 350° F. 50 but not above the boiling point of the oil.

2. A lubricating oil composition formed mainly of a hydrocarbon lubricating oil which contains an alkali soap in effective amount less than 1/2% by weight, the composition having the same order of viscosity as the said hydrocarbon lubricating oil before the addition of the soap.

3. A lubricating oil composition formed mainly of a hydrocarbon lubricating oil 60 containing an alkali base soap in effective amount less than 1/2% by weight.

4. A lubricating oil composition formed mainly of a hydrocarbon lubricating oil containing a sodium soap in effective amount 65 less than 1/2% by weight.

5. A lubricating oil composition formed mainly of a hydrocarbon lubricating oil containing about 1/8% by weight of an alkali metal soap of a fatty acid.

6. A lubricating oil composition formed mainly of a hydrocarbon lubricating oil containing an alkali metal-fatty acid soap in effective amount less than 1/2% by weight.

7. A lubricating oil composition formed 75 mainly of a hydrocarbon lubricating oil containing about 1/8% by weight of a hard, white, alkali metal soap of substantial purity.

8. A lubricating oil composition formed 80 mainly of a hydrocarbon lubricating oil having a Saybolt viscosity of about 285 at 100° F., and containing an alkali metal soap in effective amount less than 1/2% by weight.

9. A lubricating oil composition formed mainly of a hydrocarbon lubricating oil containing an alkali soap in amount and physical condition adapted to increase the film-maintaining property of the oil without undesirably increasing the ash content 90 of the oil, the finished composition and the original oil having the same order of viscosity.

ARMAN E. BECKER.